

March 13, 1934.

E. A. WEAVER

1,951,043

COLOR PHOTOGRAPHY

Filed Jan. 31, 1930



Fig. 1

Fig. 2

Inventor  
Eastman A. Weaver  
By Robert Cushman & Woodbury  
his Attorneys

## UNITED STATES PATENT OFFICE

1,951,043

## COLOR PHOTOGRAPHY

Eastman A. Weaver, Winchester, Mass., assignor,  
by meane assignments, to Technicolor, Inc.,  
New York, N. Y., a corporation of Delaware

Application January 31, 1930, Serial No. 425,013

15 Claims. (Cl. 95—2)

This invention relates to composite photographic film comprising a plurality of separable films, and is particularly applicable to motion picture film provided with a plurality of emulsions adapted to record superposed images for use in producing colored pictures.

One of the objects of this invention is to provide a composite film comprising a pair of films with their emulsion sides placed face to face 10 and joined by adhesive which does not itself cause any appreciable dispersion of light, but which serves to exclude air from between the emulsions and thus prevents the refraction caused by presence of air between adjacent sepa- 15 rately-supported emulsions.

Another object is to provide a composite film of this kind which may readily be separated into its constituent films by rupture of the adhesive without damage to the emulsions, and preferably 20 without the necessity for treatment of the adhesive preparatory to such separation.

A further object is to provide composite films of this kind in which the adhesive may be readily removed upon separation of the film and to provide improved ways of removing the adhesive. 25

My invention includes also an improved art of making photographic negatives and has for an object to provide a way of adhesively joining two or more elements of a composite film for 30 perforation, winding, exposure, or storage, whereby the film may easily be separated for development without the necessity of treating the film with chemicals which are injurious to the celluloid supports of the film, or of prolonged soaking 35 of the composite film with water preparatory to separation.

Other objects of my invention will be apparent from the following explanation and from the accompanying drawing which illustrates, diagrammatically and by way of example, two photographic films made according to my invention. 40

Fig. 1 is a side view of a composite photographic film produced with three emulsions; and 45

Fig. 2 is a similar view of a composite photographic film provided with two emulsions.

The composite photographic film of Fig. 1 50 comprises two supports 11 and 12 of transparent, flexible, relatively strong material, such as celluloid, which serve to carry light sensitive emulsions 13, 14 and 16, emulsion 13 being firmly affixed to support 11, and emulsions 14 and 16 being firmly affixed to support 12.

These emulsions differ in sensitiveness to certain colors, and a preferable arrangement is to 55 utilize an emulsion 16 which is relatively in-

sensitive to green and red wave lengths and preferably chiefly sensitive to blue and violet wave lengths, an emulsion 14 relatively insensitive to red wave lengths and preferably chiefly sensitive to green wave lengths, and an emulsion 13 sensitive to red wave lengths. The celluloid support 12 and its two emulsions 14 and 16 constitute one separable film, while the celluloid support 11 and its attached emulsion 13 constitute another separable film. These two separable films 60 are united by adhesive 15 to hold them together during simultaneous exposure of their emulsions to light. In the drawing the arrow shows the direction of the light. An image will be recorded by the blue and violet components of the 65 light in emulsion 16, an image will be formed by the green components of the light in emulsion 14, and an image will be formed by the red components of the light in emulsion 13. If desired, color filters may be placed in front of the films 70 and/or affixed to or incorporated in one or more elements of the film, for the purpose of screening out undesired spectral ranges of light from certain emulsions. For example, if emulsions 16 and 14 are not sufficiently absorptive of the 75 green, blue and violet wave lengths of light, these wave lengths may be prevented from affecting the "red record" emulsion 13 by providing a red color filter incorporated in the entrant side of emulsion 13, in the emergent side of emulsion 80 85 14, or in both.

Such color filters are not always indispensable, however, since by utilizing emulsions which are strongly absorptive of predetermined spectral ranges of light, (usually those which form an 90 image therein) the emulsions themselves may be caused to screen from the underlying emulsions these predetermined spectral ranges of light.

While the above described arrangement of emulsions is deemed desirable one of the three 95 emulsions may be dispensed with. Such a construction is illustrated in Fig. 2 of the drawing, in which emulsion 16 is omitted, and the emulsion 14 attached directly to the celluloid support 12. In the use of this form of composite film, images 100 made up respectively of the red and green components are obtained, and the blue violet image is either omitted or, if desired, may be formed separately on another film.

The surfaces of photographic emulsions are 105 characterized by the presence of minute surface irregularities which, with the intervening air spaces, when two films are placed with their emulsion sides together, cause refraction of the light passing from one emulsion to the other. In unit- 110

ing the two films which comprise my composite film I prefer to utilize an adhesive 15, preferably of similar refractive index to the emulsions, which serves to fill up the minute indentations of the surfaces of the emulsions and thus minimize the refraction, but which does not substantially separate the two adjacent emulsions nor add substantially to the thickness of the composite film. By the use of an adhesive of this character, the diffusion of the light passing through the emulsions is markedly decreased.

In the practice of my invention I provide an adhesive 15 which has less cohesiveness and/or adhesiveness, offers less resistance to splitting of the composite film than the other elements (the supports and emulsions) of the respective films, in order that the separable superposed films may be pulled apart through rupture of the adhesive, or through separation of adhesive and emulsion, without injury to the emulsions. For this purpose I prefer to provide an adhesive which after application to the films will remain in a soft, easily ruptured condition.

I have found that the sticking together of two films with their emulsion sides face to face is facilitated if the adhesive contains an appreciable amount of water. It seems probable that the water contained in the adhesive serves to wet the surfaces of the adjacent emulsions and brings into play the adhesive properties of the gelatine itself.

If emulsions are united by being rolled forcibly into contact after application of pure water, they are likely to unite fully and permanently. I therefore provide with the water a substance preferably non-adhesive or only slightly adhesive by itself for preventing such complete and permanent union of the emulsions and reducing the adhesion to a mild and temporary degree adequate to hold the films together during perforation, rewinding, storage, exposure, etc., but insufficient to hinder unduly their later separation when desired. I prefer to employ a substance which is transparent, in thin layers, which is adapted to retain water and is miscible therewith and which is non-volatile and non-solidifying or slowly solidifying, and have found that glycerine is suitable for this use. One example of a suitable composition of the adhesive comprises 40 parts of water and 60 parts of glycerine. Further to reduce the relative water-content of the adhesive and regulate its adhesive power, a small amount of a substance having in itself adhesive properties, such for example as glucose may be added. Such adhesive mixture or solution is capable of remaining in a viscous or fluid condition. The adhesive since viscous or fluid is naturally weaker than the emulsions and supports of the films, and the composite film thus temporarily joined may easily be separated without injury to the emulsions and without preliminary treatment, such for example as soaking. Vacuum probably plays a part in such adhesion, as gelatine absorbs water with such avidity as to produce actual suction if the supply is small, as it should be to avoid swelling.

In preparing composite film for motion picture use, the separate supports 11 and 12 each coated with their respective emulsions may after the application of the adhesive to one of the emulsions be brought together with their emulsion sides in contact, pressed tightly together, preferably by rolls, to insure good contact and reduce the amount of adhesive between the emulsions, and if necessary wiped free from surplus

adhesive. These operations may be performed rapidly, successively and continuously, and should be performed in darkness or in such degree of illumination as will not affect the sensitive emulsions. When ready for development the composite film may be separated by being pulled apart through rupture of the adhesive, and after separation adhesive remaining on the emulsions may be washed or squeegeed off. The separated films may be developed and used in any desired manner in the production of colored pictures. The removal of such remaining adhesive by washing may be accomplished without the use of chemicals, (which might injure the films) since the adhesive is miscible in water.

In utilizing the composite film of Fig. 1, wherein one of the separable films carries a pair of emulsions, the image in one of these emulsions may be rendered more intense than the image in the other, a print taken by projecting light through both of these images, the more intense image then removed, and a second print taken through the remaining image after rendering the latter more intense, in the manner described and claimed in Patent No. 1,808,584 to Leonard T. Troland for Color photography, of May 7, 1931. Instead of two separate emulsions, these two images may be formed in a single emulsion which has been superficially color-sensitized.

The placing of the emulsions 13 and 14 face to face with no substantial separating body or diffusion-producing layer or air space therebetween permits the light from the object photographed to form sharp images in both of these emulsions. The adhesion of the two films during handling and exposure eliminates the chance of marking of the emulsions which may result from "static," or frictional electrical discharges caused by running two emulsions together and separating them at relatively high speeds. In addition the sensitive emulsions are protected from accidental scratching or abrasion.

I may obtain some of the above described advantages and certain other advantages by employing an adhesive which does not necessarily contain water but which may be applied in such a manner as to fill the minute surface indentations without substantially separating the adjacent emulsions, which may easily be ruptured in separating the films, and after separation may be removed mechanically.

Examples of such an adhesive are rubber and transparent cements containing a gum, such as rubber, I prefer to apply such an adhesive in two stages, by first applying a preliminary coat of a thin solution of the adhesive to the emulsion surfaces of the two films and then, after drying of the originally fluid adhesive to form a tacky coating and just as the films are about to pass between the uniting rollers, applying a solvent for the adhesive, with or without some of the adhesive agent in solution, preferably only over the picture area of the films. This method of applying the adhesive insures that the edges of the films will be held firmly together, and permits the exclusion of air from between the picture areas.

After exposure, the composite film may be pulled apart through rupture of the adhesive, and the adhesive removed, if desired, by passing the emulsion side of the separated film and adhering rubber adhesive into and out of rolling contact with a surface for which the adhesive has a greater affinity than for the emulsion, for example, the surface of a rotary member of tacky

- rubber. The adhesive on the film having more affinity for the tacky rubber surface clings to this in passing, and is thus cleanly detached without injury to the emulsion.
5. Suitable solvents may if desired be employed for removing the adhesive, but I prefer the above-described method of removal since it obviates any difficulty attendant upon the remaining of solvent with traces of adhesive upon the surface of the emulsion.
- From the foregoing it will be evident that in one aspect a characteristic feature of the invention consists in that the adhesive has less internal strength than the emulsions have, so that there is no danger of rupturing the emulsions in the peeling process, and thereafter the adhesive may be removed as aforesaid without injury to the emulsions.
- I claim:
20. 1. Art of making photographic negative records which comprises joining two photographic films with emulsions face to face by means of a weak adhesive which fills the surface indentations of the emulsions without substantially separating the emulsions, exposing the combined film, separating the two films and removing the adhesive from the film.
2. Art of making photographic negative records which comprises joining two photographic films with emulsions face to face by means of a weak water miscible adhesive which fills the surface indentations of the emulsions without substantially separating the emulsions, exposing the combined film, separating the two films and removing the adhesive from the film.
3. A composite film adapted for use in color photography comprising a pair of films each coated with an emulsion, said films being superposed with their emulsions face to face, the composite film being provided between the adjacent emulsions with an easily separated adhesive which fills the minute surface indentations of the adjacent emulsions without substantially separating the emulsions whereby refraction of light passing from one emulsion to the other is minimized.
4. A composite film adapted for use in color photography comprising a pair of films each coated with an emulsion, said films being superposed with their emulsions face to face, the composite film being provided between the adjacent emulsions with water soluble easily ruptured adhesive which fills the minute surface indentations of the adjacent emulsions without substantially separating the emulsions, whereby refraction of light passing from one emulsion to the other is minimized.
5. A composite film adapted for use in color photography comprising a pair of films each coated with an emulsion, said films being superposed with emulsions face to face and the composite film being provided between the adjacent emulsions with easily ruptured adhesive offering less resistance to splitting of the composite films than the other elements thereof, whereby the superposed films may be pulled apart by rupture of said adhesive without injury to the emulsions, said adhesive being adapted to be removed from the emulsions mechanically without injury to the emulsions.
6. A composite film adapted for use in color photography comprising a pair of films each coated with an emulsion said films being superposed with their emulsions face to face, the composite film being provided between the adjacent emulsions with adhesive including water and glycerine which fills the minute surface indentations of the adjacent emulsions without substantially separating the emulsions, whereby refraction of light passing from one emulsion to the other is minimized.
7. A composite film adapted for use in color photography comprising a pair of films each coated with an emulsion, said films being superposed with their emulsions face to face, the composite film being provided between the adjacent emulsions with easily ruptured adhesive including a gum which fills the minute surface indentations of the adjacent emulsions without substantially separating the emulsions whereby refraction of light passing from one emulsion to the other is minimized.
8. A composite film adapted for use in color photography comprising a pair of films each coated with an emulsion, said films being superposed with their emulsions face to face, the composite film being provided between the adjacent emulsions with easily separated adhesive including rubber which fills the minute surface indentations of the adjacent emulsions without substantially separating the emulsions whereby refraction of light passing from one emulsion to the other is minimized.
9. A composite film adapted for use in color photography comprising a pair of films each coated with emulsion, said films being superposed with their emulsions face to face, the composite film being provided between adjacent emulsions with adhesive including water and glycerine.
10. A composite film adapted for use in color photography comprising a pair of films each coated with an emulsion, said films being superposed with their emulsions face to face, the composite film being provided between adjacent emulsions with adhesive including rubber and offering less resistance to rupture than the other elements of the composite film.
11. A composite film adapted for use in color photography comprising a pair of films each coated with an emulsion, said films being superposed with emulsion face to face and the composite film being provided between the adjacent emulsions with normally soft easily ruptured adhesive offering less resistance to splitting of the composite film than the other elements thereof, whereby the superposed films may be pulled apart by rupture of said adhesive without injury to the emulsions.
12. A composite film adapted for use in color photography comprising a pair of films each coated with an emulsion, said films being superposed with emulsions face to face and the composite film being provided between the adjacent emulsions with normally soft easily ruptured adhesive offering less resistance to splitting of the composite films than the other elements thereof, whereby the superposed films may be pulled apart by rupture of said adhesive without injury to the emulsions, said adhesive being soluble in water, whereby upon separation of the film said adhesive may be removed from the emulsion by water.
13. Art of removing an adhesive from the emulsion face of a photographic film without injury to the emulsion which comprises moving the film into and out of contact with a tacky rubber surface for which the adhesive has a greater affinity than for the emulsion, whereby the adhesive clings to said surface and is detached from the emulsion.

14. Art of removing an adhesive containing a gum from the emulsion face of a photographic film without injury to the emulsion, which comprises moving the film into and out of contact with a surface substantially immovable relative to said film and for which the adhesive has a greater affinity than for the emulsion, whereby the adhesive clings to said surface and is detached from the emulsion. 80
15. Art of making photographic negative records which comprises joining two photographic films with emulsions face to face by means of an adhesive which fills the surface indentations of the emulsions without substantially separating the emulsions and offers less resistance to rupture than the other elements of the composite film, exposing the combined film, separating the two films and removing the adhesive from the emulsions without injury to the same by moving the film into and out of contact with a surface for which the adhesive has a greater affinity than for the emulsions, whereby the adhesive clings to said surface and is detached from the emulsions. 85
- EASTMAN A. WEAVER. 90
- 15 90
- 20 95
- 25 100
- 30 105
- 35 110
- 40 115
- 45 120
- 50 125
- 55 130
- 60 135
- 65 140
- 70 145
- 75 150